# EUROPEAN PATENT SPECIFICATION

(11) **EP 0 110 630 B1**
(45) Date of publication and mention of the grant of the patent: **19.07.1989**
(21) Application number: 83307025.3
(22) Date of filing: 17.11.1983
(51) Int. Cl.: B22F 3/18

(54) **Production of metal strip from powder material**
Verfahren zur Herstellung eines Metallbandes aus Pulvermaterial
Fabrication d'une bande métallique à partir de matériau pulvérulent

(30) Priority: 18.11.1982 GB 8232966
(43) Date of publication of application: 13.06.1984
(73) Proprietor: THE ELECTRICITY COUNCIL, London, SW1P 4RD (GB); DAVY McKEE (SHEFFIELD) LIMITED, Sheffield S9 4EX Yorkshire (GB)
(72) Inventor: Donnelly, Martin, Handsworth Sheffield S13 9QY (GB); Dyos, Gordon Thomas, Llandegla Clwyd (GB); Warren, Philip Hearn, Chester Cheshire CH2 1HH (GB); Winstanley, Raymond, Ness S. Wirral L64 4AZ (GB)
(74) Representative: Cross, Rupert Edward Blount

(56) References cited:
- DE-B- 2 200 971
- GB-A- 1 039 548
- GB-A- 1 380 335
- US-A- 2 935 402

## Description

This invention relates to the production of metal strip from powder material.

It is known to compact metal powder into a "green" strip by cold pressing using rolls and then to pass the strip so formed through a sintering furnace to increase the bond between individual particles.

The cold compacted green strip typically has a density of the order of 85% ofthe full density ofthe metal and thus further processing, normally involving a further heating operation, has usually been considered necessary if a dense, non-porous product is to be obtained. The green strip is brittle and will readily fracture under tensile forces. Thus problems arise in handling this strip in order to effect the heat treatment which, in conventional furnaces, requires a long furnace within which the strip must be supported whilst subjected to the minimum of tensile stress.

It has been proposed in specification GB-A-1488007 to form the green strip by compacting metal powder and then to heat the strip in a non-oxidising atmosphere by heat transfer thereto from a bath of molten metal through which a strip is passed whilst moving it in the direction of its length and applying further compaction or consolidation to the heated strip. The molten metal bath provides not only heat transfer to the strip but also serves to support the strip as it passes therethrough.

It has also been proposed in GB-A-1380335 to form the green strip by compacting metal powder between forming rolls and then sintering the strip by heating with electron gun heating devices in an evacuated enclosure. The strip is supported on moving belts during the sintering process. After sintering the strip may be hot or cold rolled before passing out of the evacuated enclosure through a sealing arrangement to be collected on a spool.

US-A-2935402 discloses a process for converting metal powders into compacted strips or the like. The powder is initially heated, whilst held on a suitable support, to form a fairly self-sustaining, bar or slab. This partly compacted porous bar is then passed through a second furnace and hot rolled to achieve a high degree of densification.

In one aspect, the present invention provides a method of manufacturing dense metal strip from an unsintered green compacted powder strip of less than full density, which comprise the steps of, in a chamber containing a gaseous atmosphere at sub-atmospheric pressure suitable for operating a glow discharge electron beam device, passing the strip continuously through heating means comprising one or more glow discharge heating devices to heat the strip up to a temperature suitable for hot rolling, and subsequently passing the strip into a rolling mill within said chamber, characterised in thatthe rolling mill has two stages which effect the required compaction of the strip immediately after heating, a further glow discharge heating device is provided for reheating the strip between thetwo stages, and in that the strip is heated to a temperature less than that required for sintering.

Effecting the required further compaction of the strip in this way by hot rolling requires a lower temperature than sintering and it is thus possible to feed the green strip through the heating means and into the rolling mill although the green strip is very brittle and fragile.

The heating means conveniently comprises a plurality of glow discharge guns which may be, for example, as described in GB-A-2050044. It is possible, using such devices to have a very short furnace through which the green strip can be fed with negligible tension on the strip, particularly if positive feed means are provided driving the strip into the heating means from a coil of the strip material. In some cases it may be convenient to use radiant heating means in addition to glow discharge guns. These glow discharge heating means are particularly convenient in enabling the process to be carried out at a very low ambient atmospheric pressure. Using the glow discharge gun or guns, the whole chamber is evacuated to a sufficiently low pressure such that the required glow discharge can be produced.

The atmosphere employed in said chamber will be chosen in accordance with the metal being processed. Commonly a non-oxidising atmosphere will be desired and for example hydrogen may be used in the processing of metals such as stainless steel.

Preferably the strip is fed into said heating means from a coil of the green strip material in said chamber and, after said further compaction, is then coiled in said chamber.

If a hot strip is to be coiled in said chamber, problems can arise because of successive turns of the coil adhering to one another and/or because of thermal contraction of the strip on cooling. Forthis reason, if the strip is coiled whilst hot, it is preferred to interleave a layer of refractory flexible material, e.g. a ceramic paper, between successive turns of the coiled metal strip. Conveniently a ceramic fibre paper material, e.g. an alumina fibre material, is employed for this purpose.

The invention includes within its scope a metal strip produced by the above-described method.

Furthermore, in another aspect, the invention provides an apparatus for the manufacture of dense metal strip from an unsintered green compacted powder strip of less than full density, comprising a chamber for containing a gaseous atmosphere at a sub-atmospheric pressure, glow discharge heating means in the chamber to heat the strip up to a temperature which is suitable for hot rolling and a rolling mill in the chamber for rolling the strip after leaving the heating means, characterised in that the rolling mill has two stages arranged to effect the required compaction of the strip immediately after heating, and a further glow discharge heating device is provided for reheating the strip between the two stages, the glow discharge heating means being adapted to heat the strip to a temperature below that required for sintering.

There may be provided, preferably within the chamber, means for carrying the green strip as a coil with drive means for feeding the strip into the heating means. Positive driving to feed the strip into the heating means enables the tension to be kept low as the strip is being heated.

Means may be provided for coiling said strip in said chamber as it leaves the rolling mill. These means may include means for interleaving a layer of refractory flexible material between the successive turns of the coiled metal strip.

The following is a description of one embodiment of the invention, reference being made to the accompanying drawing which is a front elevation view, with the front cover removed, of a chamber containing apparatus for making stainless steel strip from a compacted powder strip.

Referring to the drawing, a chamber 10 is provided with means, not shown, for evacuating the chamber to a low pressure suitable for the operation of glow discharge guns. The residual atmosphere is chosen in accordance with the type of metal of which the strip is formed. In this particular example, the strip is of stainless steel and the residual atmosphere is hydrogen. The pressure is at the required low pressure suitable for maintaining a glow discharge. At this pressure of hydrogen, any residual oxygen will be well below the critical level and there will be no oxidising of the metal on heating.

The green strip is loaded into the chamber as a coil 11, the end of which extends from the coil, as shown at 12, partially around a drive capstan 13 which provides a positive feed for the strip feeding it into a heating system comprising, in this particular embodiment five successive glow discharge guns 14 to 18. Each of these guns is of the kind described in GB-A-2050044 and reference may be made to that specification for a full description of suitable heating devices.

From the heating system, the strip is fed to a rolling mill containing two stages formed by rolls 20 and rolls 22 which effect the required compaction of the heated strip. The compaction is effected immediately after heating so minimising any cooling before the strip enters the mill. A further glow discharge device 21 is provided for reheating of the strip between the two stages. Compaction of powdered material in this way can be effected at a lower temperature than is required for sintering and it is thus possible to feed the green strip through the heating means and into the rolling mill although the green strip itself is very brittle and fragile. The compaction forms the strip into a dense metal strip which can be fed, as shown at 23, through a strip guide 24 to a take-up spool 25.

It may be desirable, in some cases, to interleave a flexible and resilient refractory strip (e.g. a ceramic paper) between the turns of the metal as the metal is fed onto the take-up spool 25. This refractory strip becomes compressed on cooling of the metal but keeps the turns separate and permits of contraction of the metal.

With the apparatus described above, having the rolling mill in a vacuum chamber, oxidation of the rolls is avoided and it is unnecessary to use a lubricant (such as water) as in conventional hot metal rolling.

## Claims

1. A method of manufacturing dense metal strip from an unsintered green compacted powder strip of less than full density, which comprise the steps of, in a chamber containing a gaseous atmosphere at sub-atmospheric pressure suitable for operating a glow discharge electron beam device, passing the strip continuously through heating means comprising one or more glow discharge heating devices to heat the strip up to a temperature suitable for hot rolling, and subsequently passing the strip into a rolling mill within said chamber, characterised in, that the rolling mill has two stages which effect the required compaction of the strip immediately after heating, a further glow discharge heating device is provided for reheating the strip between the two stages, and in that the strip is heated to a temperature less than that required for sintering.

2. A method as claimed in claim 1 wherein the strip is fed into said heating means from a coil of the green strip material in said chamber and, after said further compaction, is then coiled in said chamber.

3. A method as claimed in claim 1 wherein radiant heating is used in addition to glow discharge heating.

4. A method as claimed in claim 1 wherein the atmosphere in said chamber is a non-oxidising atmosphere.

5. A method as claimed in claim 4 wherein the atmosphere in said chamber is hydrogen.

6. A method as claimed in claim 2 wherein the strip is coiled with an interleaved layer of refractory flexible material.

7. A method as claimed in claim 6 wherein the refractory flexible material is a ceramic paper.

8. Apparatus for the manufacture of dense metal strip from an unsintered green compacted powder strip of less than full density, comprising a chamber (10) for containing a gaseous atmosphere at a sub-atmospheric pressure, glow discharge heating means (14-18) in the chamber to heat the strip up to a temperature which is suitable for hot rolling and a rolling mill (20, 22) in the chamber for rolling the strip after leaving the heating means, characterised in that the rolling mill has two stages (20, 22) arranged to effect the required compaction of the strip immediately after heating, and a further glow discharge heating device (21) is provided for reheating the strip between the two stages, the glow discharge heating means being adapted to heat the strip to a temperature below that required for sintering.

9. Apparatus as claimed in claim 8 wherein the heating means comprise a plurality of glow discharge guns (14-18).

10. Apparatus as claimed in claim 8 and having means (11) in said chamber for carrying the green strip as a coil with drive means (13) for feeding the strip into the heating means and means (25) for coiling said strip in said chamber as it leaves the rolling mill.

11. Apparatus as claimed in claim 10 wherein the means for coiling the strip include means interleaving a layer of refractory flexible material between the successive turns of the coiled metal strip.

## Patentansprüche

1. Verfahren zum Herstellen eines dichten Metallbandes aus einem nichtgesinterten, verdichteten Rohpulverband mit weniger als der vollen Dichte, welches die Sschritte umfaßt: in einer Kammer, die eine Gasatmosphäre auf einem unter dem Außenluftdruck liegenden Druck enthält, die zum Betrieb einer Glühentladeelektronenstrahlvorrichtung geeignet ist, erfolgendes ununterbrochenes Führen des Bandes durch Heizeinrichtungen, die eine oder mehrere Glühentladeheizvorrichtungen umfassen, um das Band auf eine Temperatur aufzuheizen, die für ein Heißwalzen geeignet ist, und anschließendes Führen des Bandes in ein Walzwerk in der Kammer, dadurch gekennzeichnet, daß das Walzwerk zwei stufen hat, die die gewünschte Verdichtung des Bandes unmittelbar nach dem Heizen bewirken, eine weitere Glühentladeheizvorrichtung vorgesehen ist, um das Band zwischen den beiden stufen wieder aufzuheizen und das Band auf eine Temperatur unter derjenigen Temperatur aufgeheizt wird, die zum Sintern erforderlich ist.

2. Verfahren nach Anspruch 1, bei dem das Band in die Heizeinrichtungen von einem Coil des Rohbandmaterials in der Kammer eingegeben und nach der weiteren Verdichtung in der Kammer anschließend aufgewickelt wird.

3. Verfahren nach Anspruch 1, bei dem eine Strahlungsheizung zusätzlich zur Glühentladeheizung benutzt wird.

4. Verfahren nach Anspruch 1, bei dem die Atmosphäre in der Kammer eine nicht oxidierende Atmosphäre ist.

5. Verfahren nach Anspruch 4, bei dem die Atmosphäre in der Kammer Wasserstoff ist.

6. Verfahren nach Anspruch 2, bei dem das Band mit einer zwischengelegten Sschicht aus einem feuerfesten flexiblen Material aufgewickelt wird.

7. Verfahren nach Anspruch 6, bei dem das feuerfeste flexible Material ein keramisches Papier ist.

8. Vorrichtung zum Herstellen eines dichten Metallbandes aus einem nichtgesinterten verdichteten Rohpulverband mit weniger als der vollen Dichte mit einer Kammer (10) zum Aufnehmen einer Gasatmosphäre auf einem Druck unter dem Außenluftdruck, Glühentladeheizeinrichtungen (14,18) in der Kammer zum Aufheizen des Bandes auf eine Temperatur, die zum Heißwalzen geeignet ist, und einem Walzwerk (20, 22) in der Kammer zum Walzen des Bandes nach dem Verlassen der Heizeinrichtungen dadurch gekennzeichnet, daß das Walzwerk zwei stufen (20, 22) hat, die so angeordnet sind, daß sie die erforderliche Verdichtung des Bandes unmittelbar nach dem Heizen bewirken, und daß eine weitere Glühentladeheizvorrichtung (21) vorgesehen ist, um das Band zwischen den beiden stufen wieder aufzuheizen, wobei die Glühentladeheizeinrichtungen so ausgebildet sind, daß sie das Band auf eine Temperatur unter derjenigen Temperatur aufheizen, die zum sintern erforderlich ist.

9. Vorrichtung nach Anspruch 8, bei der die Heizeinrichtungen eine Vielzahl von Glühentladekanonen (14-18) umfassen.

10. Vorrichtung nach Anspruch 8, mit Einrichtungen (11) in der Kammer zum Tragen des Rohbandes als Coil mit einer Antriebseinrichtung (13) zum Einführen des Bandes in die Heizeinrichtungen und Einrichtungen (25) zum Aufwickeln des Bandes in der Kammer, wenn es das Walzwerk verläßt.

11. Vorrichtung nach Anspruch 10, bei der die Einrichtungen zum Aufwickeln des Bandes Einrichtungen einschließen, die eine schicht aus einem feuerfesten flexiblen Material zwischen die aufeinanderfolgenden Wicklungen des aufgewikkelten Metallbandes legen.

## Revendications

1. Procédé de fabrication d'une bande métallique dense à partir d'une bande de poudre compactée verte non frittée d'une densité inférieure à la pleine densité, qui comprend les étapes de, dans une chambre contenant une atmosphère gazeuse à pression subatmosphérique convenant au fonctionnement d'un dispositif à faisceau d'électrons à décharge luminescente, passage de la bande de façon continue par des moyens de chauffage comprenant un ou plusieurs dispositifs de chauffage à décharge luminescente pour chauffer la bande jusqu'à une température convenant à un laminage à chaud, et ensuite passage de la bande dans un laminoir à l'intérieur de ladite chambre, caractérisé en ce que le laminoir comporte deux cages qui effectuent le compactage requis de la bande immédiatement après le chauffage, un dispositif supplémentaire de chauffage à décharge luminescente est prévu pour réchauffer la bande entre les deux cages, et en ce que la bande est chauffée jusqu'à une température inférieure à celle requise pour le frittage.

2. Procédé selon la revendication 1 dans lequel la bande est introduite dans lesdits moyens de chauffage à partir d'une bobine du matériau en bande verte dans ladite chambre et, après ledit compactage supplémentaire, est alors bobinée dans ladite chambre.

3. Procédé selon la revendication 1 dans lequel un chauffage à rayonnement est utilisé en plus du chauffage à décharge luminescente.

4. Procédé selon la revendication 1 dans lequel l'atmosphère dans ladite chambre est une atmosphère non-oxydante.

5. Procédé selon la revendication 4 dans lequel l'atmosphère dans ladite chambre est de l'hydrogène.

6. Procédé selon la revendication 2 dans lequel la bande est bobinée avec une couche intercalée de matériau flexible réfractaire.

7. Procédé selon la revendication 6 dans lequel le matériau flexible réfractaire est un papier céramique.

8. Appareil pour la fabrication d'une bande métallique dense à partir d'une bande de poudre compactée verte non frittée d'une densité inférieure à la pleine densité, comprenant une chambre (10) pour contenir une atmosphère gazeuse à pression subatmosphérique, dea moyens de chauffage à décharge luminescente (14-18) dans la chambre pour chauffer la bande jusqu'à une température qui convient à un laminage à chaud et un laminoir (20, 22) dans la chambre pour laminer la bande une fois qu'elle a quitté les moyens de chauffage, caractérisé en ce que le laminoir comporte deux cages (20, 22) agencés pour effectuer le compactage requis de la bande immédiatement après le chauffage, et un dispositif supplémentaire de chauffage à décharge luminescente (21) est prévu pour réchauffer la bande entre les deux cages, les moyens de chauffage à décharge luminescente étant adaptés pour chauffer la bande jusqu'à une température inférieure à celle requise pour le frittage.

9. Appareil selon la revendication 8 dans lequel les moyens de chauffage comprennent plusieurs canons à décharge luminescente (14-18).

10. Appareil selon la revendication 8 et comportant un moyen (11) dans ladite chambre pour porter la bande verte en une bobine avec un moyen d'entraînement (13) pour introduire la bande dans les moyens de chauffage et un moyen (25) pour bobiner ladite bande dans ladite chambre au fur et à mesure qu'elle quitte le laminoir.

11. Appareil selon la revendication 10 dans lequel le moyen pour bobiner la bande comprend un moyen intercalant une couche de matériau flexible réfractaire entre les tours successifs de la bande métallique bobinée.
